

## UNITED STATES PATENT OFFICE

2,393,594

## OPERATION OF INTERNAL-COMBUSTION ENGINES

Clyde O. Davis, Woodbury, N. J., assignor to E. I. du Pont de Nemours & Company, Wilmington, Del., a corporation of Delaware

No Drawing. Application July 8, 1941,  
Serial No. 401,547

2 Claims. (Cl. 123—1)

This invention relates to a novel method for the production and utilization of energy and more particularly to a method for the operation of internal combustion engines.

Internal combustion engines are highly efficient sources of mechanical power and can be broadly divided into two classes, those in which both the fuel and oxidant are introduced into the combustion chamber in vaporous form and those into which the fuel is injected in finely divided but non-vaporous form, because of the practical difficulties in vaporizing the fuel. The two foregoing types are represented by the ordinary gasoline engine and the Diesel engine, respectively. With such engines, the oxygen of the air serves for the combustion of the fuel, since air is generally available free, uncompressed. In certain cases, however, internal combustion engines are operated in places where there is a deficiency of available air or oxygen, or where at least the supply is limited. Such conditions would hold, for example, in stratosphere flights and on board submarines, and the maintenance at hand of a reservoir of highly combustible fuel might also be undesirable at times, as in wartime use under conditions of exposure to shell fire.

The object of the present invention is a novel method of producing and utilizing energy by use of an internal combustion engine. A further object is a method for the operation of internal combustion engines which does not require an extensive supply of gaseous oxidizing agents for the combustion of the fuel. A still further object is a method for the operation of internal combustion engines wherein both fuel and oxidizing agent are introduced in solution form. Additional objects will be disclosed as the invention is described more in detail hereinafter.

I have found that the foregoing objects are obtained when I introduce into the combustion chamber of an internal combustion engine a solution comprising ammonium nitrate and an oxidizable material and bring about the combustion of the oxidizable material therein. Several types of solutions may be employed according to the invention. I may, for example, dissolve ammonium nitrate in liquid ammonia and use such a solution, the ammonia being burnt in the available oxygen of the ammonium nitrate. Alternatively, I may employ an aqueous solution of ammonium nitrate, said solution containing also a dissolved combustible material. While such solutions are the ones that will preferably be employed, my invention contemplates the use

of any ammonium nitrate solution, whatever the solvent, where an oxidizable material is present either as solvent or as an additional solute. It will be apparent that additional oxidizing agents may be present also, along with the ammonium nitrate.

Since the dissolved ammonium nitrate is a very considerable part of the combustion mixture and since other dissolved solids may be present also, 10 it will be apparent that the most suitable type of internal combustion engine for use will be one in which the solution is injected in finely divided form. It will be applicable, for example, in the Diesel engine type, whether of the simple compression type or the semi-Diesel type where spark ignition is employed.

While ammonium nitrate is the principal oxidizing agent present, and is particularly desirable because no solid residue remains after combustion, 20 additional oxidants may be used also, such as soluble chromates or dichromates, permanganates, alkali nitrates or nitrites, and the like. Such materials as nitrous oxide may be present also, either in liquid or in vaporous form.

25 Likewise, the combustible material may vary widely, either as solvent for the ammonium nitrate or as additional dissolved material. One of my preferred materials is anhydrous liquid ammonia which is a solvent for ammonium nitrate, forming the so-called Diver's solution. Methyl and ethyl alcohols may likewise be employed as a portion of the solution, mixed with liquid ammonia, if desired. Additional solvents capable of application, as the entire solvent or portion 30 thereof, are pyridine, acetone, formamide, dimethylformamide, and the like. The combustible may also be a dissolved material, especially when aqueous solutions of ammonium nitrate are used. The dissolved material may consist of such substances as sugar, urea, diphenylamine, and many others.

35 It will be understood that various additional materials, which essentially are neither oxidants nor combustible materials, may be desirable additions under certain conditions, as combustion accelerants or retardants, knock suppressants, ignition point depressants, and the like.

40 Various blends of combustible and oxidizing agent were applied successfully in a 4-cycle vertical type Diesel engine. These included a 91-19 solution, by weight, of ammonium nitrate in liquid ammonia, an 80-20 ammonium nitrate-ammonia mixture blended with methyl alcohol in various proportions, a 50-50 blend of dimethylformamide and the foregoing Diver's solution.

together with a small amount of ethyl nitrate, ammonium nitrate dissolved in dimethylformamide in a 30-70 ratio, and others.

The present invention is applicable to internal combustion engines generally. It will be understood that this includes not only those engines which employ the reciprocating motion of pistons, as in the Diesel engine, but also the gas turbine type of engine, in which rotary motion and impeller vanes are used. I intend the invention to cover the process described when applied to any motor in which the fuel is burnt in the combustion chamber thereof with utilization of the combustion gases.

The invention has been described in its essentials in the foregoing. It will be understood, how-

ever, that various departures may be made from the details of compositions and operations without going outside the scope of the invention. I intend to be limited therefore only by the following patent claims.

I claim:

1. The method of producing and utilizing energy, which comprises introducing into the combustion chamber of an internal combustion engine a solution of ammonium nitrate in liquid ammonia and effecting therein the explosive combustion of said ammonia.

2. A fuel for internal combustion engines comprising ammonium nitrate dissolved in liquid ammonia.

CLYDE O. DAVIS.